

July 17, 1951

H. H. HOMER

2,560,953

ELECTRIC GASEOUS DISCHARGE DEVICE ELECTRODE

Filed June 30, 1949



Fig. 1



Fig. 2

INVENTOR.  
Horace H. Homer  
BY Lawrence Burns,

ATTORNEY

## UNITED STATES PATENT OFFICE

2,560,953

ELECTRIC GASEOUS DISCHARGE DEVICE  
ELECTRODEHorace H. Homer, Arlington, Mass., assignor to  
Sylvania Electric Products Inc., Salem, Mass., a  
corporation of Massachusetts

Application June 30, 1948, Serial No. 102,304

2 Claims. (Cl. 313—178)

1

This invention relates to electric gaseous discharge devices and more particularly to fluorescent lamps.

In the manufacture of electric gaseous discharge devices, and more particularly in the manufacture of fluorescent lamps of the "hot cathode" type, i. e., those in which the electrode comprises a coiled filament of tungsten wire, such as that shown in U. S. Patent 2,258,158, for example, the electrodes are usually provided with a coating of an electron-emissive material. In the case of a fluorescent lamp electrode, the electron-emissive material usually comprises an oxide of one or more of the alkaline earth metals. For convenience, the alkaline earth metals are usually applied in the form of a carbonate which breaks down to the oxide when the lamp is processed.

During the operating life of fluorescent lamps, an objectionable discoloration frequently appears on the wall of the lamp near the ends thereof and in proximity to the electrodes. One form which this discoloration may assume is a light yellow, brownish or black ring or band which usually extends completely around the periphery of the inner wall of the lamp. This particular discoloration is usually defined by a sharp edge on the side near the electrode and a diffused edge on the side near the longitudinal center of the lamp. These rings or bands are usually found forward of the electrodes with the sharp edge located adjacent to an end of the positive column or plasma.

An object of this invention is to retard the development of this discoloration.

Further objects, advantages and features will be apparent from the following description when read in conjunction with the accompanying drawing in which:

Figure 1 is a side elevational view of a fluorescent lamp with an end thereof broken away, showing the electrode mount structure.

Figure 2 is an enlarged fragmentary detail of the electrode mount structure shown in Figure 1.

In Figure 1, the lamp 1 comprises an elongated tubular glass envelope 2, the inner wall of which is provided with a coating 3 of fluorescent material, and electrode mounts 4 (one of which is shown) sealed in the ends thereof. Each electrode mount comprises a glass stem 5 having a flared portion 6 which is sealed to the glass envelope 2, a press 7 through which lead wires 8 are sealed, and a filamentary electrode 9 of tungsten wire mounted on the lead wires. At least one of the stems 5 is provided with an aperture 55

2

10 therein to which an exhaust tube (not shown) is connected to permit evacuation of the lamp envelope during processing. The sealed envelope is provided with a filling of inert gas at low pressure, such as argon at about 3 mm. and a small quantity of mercury 11.

15 The filamentary electrode 9 is a tungsten wire which has been coiled once to define a primary coil and then a portion thereof intermediate the ends is coiled again to define a secondary coil. A quantity of electron emissive material 12, such as an oxide of one or more of the alkaline earth metals, is disposed primarily within the turns of that portion of the primary coil which has been provided with a secondary coiling. The electrode 9 is supported on lead wires 8 by clamping or welding the lead wires 8 to the ends or legs 13 of the primary coil thereof.

20 I have discovered that the development of discoloration on the wall of the lamp envelope during life can be arrested substantially by providing the legs 13 of the filamentary electrode with a reservoir of powdered zirconium 14 preferably disposed within the turns thereof. Table I below illustrates this quite clearly. This table reflects the results of a test in which the legs of the filamentary electrodes of several lamps were provided with the powdered zirconium and the legs of the filamentary electrodes of several other lamps were not so provided. The former are identified as "Zr lamps"; the latter as "controls." The discoloration at the end of various hours of burning is in terms of arbitrary relative units.

Table I

|  | Discoloration at— | 100 Hours     | 500 Hours | 875 Hours |
|--|-------------------|---------------|-----------|-----------|
|  |                   | Zr Lamps..... | 0         | 2.5       |
|  | Controls.....     | 0             | 23.3      | 43.3      |

35 I have found that the location of the powdered zirconium on the filamentary electrode mount is quite critical. For example, when powdered zirconium is placed on the lead wires instead of on the legs of the filamentary electrode, the lamps are hard to start, their brightness is diminished, and the color of the light emitted is affected.

40 Although the specific embodiment of my invention as described above and shown in the drawing is with reference to a filamentary electrode having a primary coil and a secondary coil, filamentary electrodes having a primary coil only, filamentary electrodes having primary, secondary and tertiary coiling, for example, may be employed without departing from the spirit of

my invention, viz., providing the legs of the filamentary electrode with a reservoir of powdered zirconium.

Although the powdered zirconium is shown in Figure 2 as being disposed along substantially the entire length of the legs of the filamentary electrode, beneficial effects may be obtained by locating the powdered zirconium only on that portion thereof which is inside or outside the point at which the lead wires are clamped thereover.

The powdered zirconium is applied to the legs of the filamentary electrode in the form of a suspension thereof in a suitable medium. For example, it may be prepared by adding powdered zirconium to a solution of borated silica in isopropyl alcohol.

The borated silica, hereinafter referred to as solution A, is prepared by adding an excess of anhydrous  $B_2O_3$  to isopropyl alcohol, agitating in a closed vessel for about 24 hours, and filtering. The filtered solution should contain not less than .03 gram  $B_2O_3$  per cc. of alcohol. This is solution A.

A second solution, hereinafter referred to as solution B, is prepared by slowly heating 100 cc. of ethyl silicate with 40 cc. of .6N HCl and constantly stirring the same until completion of the reaction. Completion of the reaction has been effected when the initial two phase solution becomes one phase; at the same time there is an evolution of heat and fine bubbles. Solution A is then added in the ratio of three parts of solution A to one part of this solution. This mixture is then permitted to stand for about 24 hours and is then decanted. The decanted solution is solution B.

The solution of powdered zirconium, which is applied to the legs of the electrode, is prepared by adding powdered zirconium to a mixture of solution A and solution B in the following pro-

portions: powdered zirconium 500 grams; solution A 110 cc. and solution B 40 cc. However other suitable suspension media and binders may be employed without departing from the spirit of the invention.

In the preferred embodiment of my invention the suspension of powdered zirconium is uniformly distributed and completely fills the interstices of the legs of the electrode. However, this condition is not necessary for the attainment of all the beneficial effects of my invention.

What I claim is:

1. An electric gaseous discharge device electrode comprising: a tungsten filament having coiled legs, and a coiled coil portion intermediate the legs; a quantity of electron-emissive material on said coiled coil portion; and a quantity of powdered zirconium within the interstices of said coiled legs only of said filament.
- 15 2. An electric gaseous discharge device comprising: an elongated sealed glass envelope; a filling of inert gas at low pressure in said envelope; a small quantity of mercury in said envelope; a tungsten filament in said envelope at each end thereof, each filament having coiled legs and a coiled coil portion intermediate the legs; a quantity of electron-emissive material on said coiled coil portion; and a quantity of powdered zirconium within the interstices of said 30 coiled legs only of said filament.

HORACE H. HOMER.

#### REFERENCES CITED

The following references are of record in the file of this patent:

#### UNITED STATES PATENTS

| Number    | Name         | Date          |
|-----------|--------------|---------------|
| 2,208,987 | Kuhne et al. | July 23, 1940 |
| 2,329,126 | Lemmers      | Sept. 7, 1943 |
| 2,462,837 | Braunsdorff  | Mar. 1, 1949  |